

# UNITED STATES PATENT OFFICE.

CHARLES J. REED, OF PHILADELPHIA, PENNSYLVANIA.

## METALLIC COMPOSITION.

No. 874,866.

Specification of Letters Patent.

Patented Dec. 24, 1907.

Application filed March 23, 1906. Serial No. 307,697.

To all whom it may concern:

Be it known that I, CHARLES J. REED, a citizen of the United States, residing in Philadelphia, county of Philadelphia, Pennsylvania, have invented certain new and useful Improvements in Metallic Compositions, of which the following is a specification.

My invention relates to a new composition of metals, designed particularly for use as a durable bearing for revolving shafts, and the like, wherein the same will be sufficiently hard to resist wear from the friction of moving parts in contact therewith and which will be sufficiently hard not to be readily worn away in use.

My improved composition consists of lead, arsenic, and copper melted together in suitable proportions for the work intended. I find the following proportions to give good results as an anti-friction bearing metal, viz.— lead, eighty-five parts by weight, arsenic, ten parts by weight, copper, one to five parts by weight.

I do not limit my invention to the proportions above stated, as they may be varied within certain limits and accomplish substantially the same results in accordance with the work or object required. I have found that for bearings for certain uses the proportion of arsenic may be very much greater than the proportion above given, and may in some cases be used with advantage to the extent of fifty, sixty or even seventy per cent. of the total mixture of lead, arsenic and copper.

In making the composition the metals are melted and mixed together in any suitable manner, and I find it advantageous, particularly where the proportion of arsenic is relatively high as compared to the lead and copper, to melt the metals and combine them in a receptacle while under pressure greater than one atmosphere to prevent volatilization of the arsenic. For anti-friction bearings the copper may in some cases be dispensed with, and the lead and arsenic be combined together by melting.

I am aware that in metallic mixtures for bearings lead has been used as the base metal and that it has been hardened by the addition of antimony, tin, copper, zinc and other metals, but I am not aware that for such use lead has been hardened by combining it with arsenic. I am also aware that lead containing a small proportion of arsenic, such as one or two per cent., has been used for the manufacture of shot, but this is an entirely different composition from mine owing to the difference in proportions and properties, and the use of the arsenic in the manufacture of such shot accomplishes an entirely different result from the arsenic in my composition, for such shot composition would not, for the purpose of bearings, resist wear and frictional heat as in my improved composition.

While I have referred to my improved composition as useful for bearings, it will be understood that the same may be used for other purposes.

Having now described my invention what I claim is:—

1. The herein described composition comprising lead, arsenic, and copper combined together.

2. The herein described composition comprising lead, arsenic and copper, the proportion of arsenic being not less than ten per cent.

3. The herein described composition comprising lead, arsenic and copper, the proportion of copper being less than the proportion of lead.

4. An anti-friction metal comprising lead, arsenic and copper, the proportion of arsenic being less than the proportion of lead and greater than the proportion of copper.

CHARLES J. REED.

Witnesses:

GUSTAF M. WESTMAN,  
T. F. BOURNE.